# EUROPEAN PATENT SPECIFICATION

(11) **EP 2 112 252 B1**
(45) Date of publication and mention of the grant of the patent: **15.07.2020**
(21) Application number: 09158839.2
(22) Date of filing: 27.04.2009
(51) Int. Cl.: C23C 28/00, C23C 4/10, C23C 4/11

(54) **A THERMAL BARRIER, AN ARTICLE WITH A THERMAL BARRIER, AND A METHOD OF APPLYING A THERMAL BARRIER TO A SURFACE**
WÄRMESPERRE, ARTIKEL MIT EINER WÄRMESPERRE UND VERFAHREN ZUM AUFTRAGEN EINER WÄRMESPERRE AUF EINE OBERFLÄCHE
BARRIÈRE THERMIQUE, ARTICLE DOTÉ D'UNE BARRIÈRE THERMIQUE ET PROCÉDÉ POUR APPLIQUER UNE BARRIÈRE THERMIQUE SUR UNE SURFACE

(30) Priority: 25.04.2008 GB 0807627
(43) Date of publication of application: 28.10.2009
(73) Proprietor: Zircotec IP Limited, Abingdon Oxfordshire OX14 1RL (GB)
(72) Inventor: McCabe, Andrew Robert, Didcot, Oxfordshire OX11 0QJ (GB)
(74) Representative: Dempster, Benjamin John Naftel

(56) References cited:
- EP-A- 1 541 808
- EP-A- 1 734 145
- WO-A-98/53113
- US-A- 4 248 440
- US-A- 4 542 111
- US-A1- 2007 140 840

## Description

This invention relates to a thermal barrier, an article with a thermal barrier and a method of applying a thermal barrier to a surface.

A known situation in which a heat shield is required is for an exhaust for a vehicle such as a car or motorcycle. The heat from the exhaust and associated engine, particularly on performance vehicles, is such that there is the potential for heat damage to surrounding components, and a risk of setting fire to combustible materials, such as dry grass, coming into contact with the system, as well as the risk of skin burns for any person coming into contact with the hot system.

There are currently two known solutions:
1. It is possible to provide mechanical casings with internal air-gap or thermal insulant, physical guards and heat shields. However, this is generally unsightly and costly. Furthermore, it takes up precious space and adds weight to the vehicle.
2. It is also possible to apply a thermal insulation material (eg. zirconia oxide) directly to the inside and/or outside of the system. This can be through painting or plasma spraying. This insulation material is unsightly in its natural form (its natural colour is white/yellow), is porous unless painted, and is susceptible to stone chips, thermal shock (from road surface water), discolouration and staining. Although discolouration and staining are not an issue when applied to hidden and protected components, it is far less acceptable where the coating is exposed and visible, for example on a car tail-pipe or motorcycle exhaust. WO98/53113 discloses the use of a plasma sprayed titanium dioxide as thermal barrier coating that is applied upon an automotive metallic article.

According to a first aspect of the present invention, there is provided an article as claimed in claim 1.

The thermal barrier of the invention is extremely tough, hard-wearing, scratch resistant, resistant to stone chips, resistant to corrosion and/or chemical attack, and is highly resistant to thermal shock.

Titanium dioxide is naturally white, but loses oxygen during the plasma spray process and as a result changes colour. The plasma sprayed ceramic coating has a satin black sheen, which could be considered more attractive than the natural white or pale colours of most ceramics. The plasma sprayed coating has the further advantage of retaining its consistent appearance when heated (unless excessively), unlike, for example, metallic exhaust pipes, which may show decolourisation.

A high level of porosity in the coating further increases the thermal resistance. The porosity may be at least 5%, preferably at least 10%. The quantity of pores may be sufficient to produce fine cracks in the ceramic, the cracks not resulting in total failure of the ceramic. The fine cracks further increase the voidage in the ceramic coating, thereby enabling the thermal resistance to be increased, without deleteriously affecting the coating to the extent that it fails and becomes detached from the surface to be coated.

Where the coating is a blend of titanium dioxide with at least one other ceramic material, preferably the coating comprises greater than about 30 wt.-% titanium dioxide. The other ceramic material may be added to change and control the properties of the barrier such as the final colour, surface finish, texture and physical properties of the barrier. Where the coating is not solely titanium dioxide, the or each other ceramic material may be any suitable ceramic material, but preferably the other ceramic material includes at least one of zirconium dioxide, chromium dioxide, aluminium oxide, and magnesium zirconate.

The thermal barrier may be of constant thickness. In an alternative embodiment, the coating may have different thicknesses in different places to provide different degrees of protection from heat. The thermal barrier is at least 100 micrometres in thickness. The thicker the coating, the better its thermal barrier properties. Preferably the thermal barrier is not more than 500 micrometres in thickness.

The article may be made of steel.

The article may include at least one intermediate layer beneath the thermal barrier. The or one intermediate layer may be of metal or metal alloy, and may be or contain nickel.

According to a second aspect of the present invention, there is provided a method as claimed in claim 10.

Thermal spraying is a desirable deposition method, as a controllable amount of porosity can be introduced into the coating. The thermal spraying is conducted by plasma spraying, and preferably by nitrogen plasma spraying.

Preferably the at least one other ceramic material comprises at least one of zirconium dioxide, chromium dioxide, aluminium oxide, and magnesium zirconate.

Preferably the surface is roughened prior to spraying of the thermal coating, for example by grit blasting. Roughening of the surface improves the chemical and physical activity of the surface, and increases the surface area, thus improving the coating bond strength.

Preferably the method further comprises applying a bond coat to the surface before applying the thermal barrier. The bond coat may be a metal or a metal alloy, and may contain nickel. The bond coat provides a more secure bond between the thermal barrier coating and the surface to be coated. In addition it minimises the effect of thermal mismatch between the surface and the ceramic top coat.

According to a further aspect of the invention there is provided the use as claimed in claim 14.

Embodiments of the invention will now be described by way of example.

### Embodiment 1

In this embodiment, a thermal barrier coating was applied to a mild steel exhaust pipe.

Before coating, the exhaust pipe was thoroughly degreased, inside and out, using acetone. Areas not requiring coating were masked off using proprietary masking tape. The pipe was grit blasted to give a rough surface, using a siphon-type grit blast system at 2.76 bar (40 psi) with 0.4 to 0.5mm aluminium oxide grit.

The roughened pipe was mounted in a rotating chuck, in a plasma spray booth equipped with a robot manipulation system. The robot was programmed to spray the rotating pipe.

A nickel based bond coat comprising nickel - 40% aluminium was plasma sprayed onto the pipe to a thickness of ∼100 µm. The plasma spray parameters used were Nitrogen 50 slpm, hydrogen 5 slpm, current 400 Amps, carrier gas 5 slpm, spray distance 100 mm, powder flow 45 g/min.

The thermal barrier coating was then applied by plasma spraying a 50/50 wt.-% mixture of titanium dioxide and magnesium zirconate on top of the bond coat. The thermal barrier coating was applied to a thickness of ∼200 µm. The plasma spray parameters used were Nitrogen 45 slpm, hydrogen 5 slpm, current 500 Amps, carrier gas 5 slpm, spray distance 75 mm, powder flow 65 g/min, ceramic powder particle size 50 to 90 micrometres. The ceramic was plasma sprayed so that the resulting coating was of graduated thickness being thicker nearer to inlet end of the exhaust pipe and thinner nearer to the outlet end.

After the coatings had been applied, the masking tape was removed, leaving a deep grey/black coating in the required areas on the pipe.

The exhaust pipe was then tested for thermal shock properties by heating to 500°C then immersing in water at 20°C, and repeating that process thirty times. The exhaust coating showed no signs of failure, and the test had no impact on its appearance. Longer term testing in which the exhaust was subject to an accelerated twenty year lifetime test, showed that the exhaust and its coating remained intact and operable, without corrosion, and still acceptable in appearance, thereby extending the operating life of the overall system.

Porosity was typically 10 %, with a thermal conductivity of 2 W/mK .

### Embodiment 2

In this embodiment, a thermal barrier coating was applied to a stainless steel heat shield.

The heat shield was prepared in the same way as the exhaust pipe in embodiment 1.

The robot was programmed to perform a ladder movement across the heat shield.

A nickel based bond coat was applied as in embodiment 1.

The thermal barrier coating was then applied by plasma spraying 100 wt.% titanium dioxide using the same parameters as in embodiment 1

The resulting thermal coating was black.

The weight increase was used to determine the coating thickness which was 200 µm

The properties were similar to those in embodiment 1.

### Embodiment 3

In this embodiment, a thermal barrier coating was applied to an exhaust manifold.

The exhaust manifold was prepared in the same way as the parts in embodiments 1 and 2.

As the exhaust manifold had a complex shape, plasma spraying was carried out using a hand held plasma spray gun.

A nickel based bond coat, of the same composition as that the bond coats used in embodiments 1 and 2 was applied as a thin even layer.

The thermal barrier coating was then applied by plasma spraying a 40/60 wt.-% mixture of fine particle size TiO₂ and Al₂O₃, namely 20 to 50 µm particle size powder. Due to the fine powder particle size, the carrier gas flow was increased to 8 slpm, the spray distance decreased to 65 mm and powder flow rate decreased to 40 g/min compared to the spray parameters in embodiments 1 and 2. The spray parameters were otherwise unchanged.

The resulting thermal barrier coating was a deep grey/black. The appearance was uneven until final cleaning took place, using a compressed air line to remove loosely bonded unmelted powder particles.

## Claims

1. An article with a thermal barrier comprising a coating of ceramic material comprising 20 to 100% wt-% titanium dioxide, wherein the thermal barrier is a plasma sprayed coating having a deep grey or black appearance, the thickness of the coating being at least 100 micrometres, the article being made of metal and being a car tail pipe or a motorcycle exhaust.

2. An article as claimed in claim 1, wherein the coating comprises a coating of titanium dioxide only.

3. An article as claimed in claim 1, wherein the coating has greater than about 30 wt.-% titanium dioxide, and preferably has at least 50 wt.-% titanium dioxide.

4. An article as claimed in claim 1, 2 or 3, wherein the coating comprises titanium dioxide and at least one other ceramic material, and the other ceramic material preferably comprises at least one of zirconium dioxide, chromium dioxide, aluminium dioxide, and magnesium zirconate.

5. An article according to any preceding claim, wherein the thermal barrier is a plasma sprayed coating.

6. An article according to any preceding claim, wherein the thermal barrier has different thicknesses in different places to provide different degrees of protection from heat.

7. An article according to any preceding claim, wherein the thermal barrier is not more than 500 micrometres in thickness.

8. An article according to any preceding claim, wherein the article is made steel.

9. An article according to any preceding claim, wherein the article includes at least one intermediate layer beneath the thermal barrier, preferably the or one intermediate layer being a metal or metal alloy, and more preferably the intermediate layer being or containing nickel.

10. A method of applying a thermal barrier to a surface of a metal article, the article being a car tail pipe or a motorcycle exhaust, the method comprising plasma spraying onto the surface a ceramic material comprising 20 to 100 wt.-% titanium dioxide to a thickness of at least 100 micrometres such that the sprayed coating has a deep grey or black appearance.

11. A method as claimed in claim 10, wherein the ceramic material comprises titanium dioxide and at least one other ceramic material, preferably at least one of zirconium dioxide, chromium dioxide, aluminium oxide, and magnesium zirconate.

12. A method according to claim 10 or claim 11, wherein the plasma spraying is nitrogen plasma spraying.

13. A method according to claim 10, claim 11, or claim 12, wherein the method further comprises applying a bond coat to the surface before applying the thermal barrier, the bond coat preferably being a metal or a metal alloy, and more preferably being or containing nickel.

14. The use of plasma sprayed titanium dioxide alone or in combination with another ceramic material at a titanium dioxide content of at least 20 wt.-% in a coating of at least 100 micrometres thickness as a thermal barrier on an article made of metal being a car tail pipe or a motorcycle exhaust, the coating being plasma sprayed so as to achieve a deep grey or black appearance.

## Patentansprüche

1. Artikel mit einer Wärmesperre, aufweisend eine Beschichtung aus Keramikmaterial, aufweisend 20 bis 100 Gew.-% Titandioxid, wobei die Wärmesperre ein dunkelgraues oder schwarzes Aussehen hat, die Dicke der Beschichtung wenigstens 100 µm beträgt, der Artikel aus Metall gefertigt ist und ein Fahrzeugauspuff oder ein Motorradauspuff ist.

2. Artikel wie in Anspruch 1 beansprucht, wobei die Beschichtung ausschließlich eine Beschichtung aus Titandioxid aufweist.

3. Artikel wie in Anspruch 1 beansprucht, wobei die Beschichtung mehr als etwa 30 Gew.-% Titandioxid hat und vorzugsweise wenigstens 50 Gew.-% Titandioxid hat.

4. Artikel wie in Anspruch 1, 2 oder 3 beansprucht, wobei die Beschichtung Titandioxid und wenigstens ein anderes Keramikmaterial aufweist, und das andere Keramikmaterial vorzugsweise wenigstens eines von Zirkoniumdioxid, Chromdioxid, Aluminiumdioxid und Magnesiumzirkonat aufweist.

5. Artikel gemäß einem der vorhergehenden Ansprüche, wobei die Wärmesperre eine plasmagespritzte Beschichtung ist.

6. Artikel gemäß einem der vorhergehenden Ansprüche, wobei die Wärmesperre an verschiedenen Stellen unterschiedliche Dicken aufweist, um unterschiedliche Hitzeschutzgrade vorzusehen.

7. Artikel gemäß einem der vorhergehenden Ansprüche, wobei die Wärmesperre nicht mehr als 500 µm dick ist.

8. Artikel gemäß einem der vorhergehenden Ansprüche, wobei der Artikel aus Stahl gefertigt ist.

9. Artikel gemäß einem der vorhergehenden Ansprüche, wobei der Artikel wenigstens eine Zwischenschicht unter der Wärmesperre aufweist, wobei die oder eine Zwischenschicht ein Metall oder eine Metalllegierung ist, und noch bevorzugter die Zwischenschicht Nickel ist oder Nickel enthält.

10. Verfahren zum Aufbringen einer Wärmesperre auf einer Oberfläche eines Artikels aus Metall, wobei der Artikel ein Fahrzeugauspuff oder ein Motorradauspuff ist, wobei das Verfahren Plasmaspritzen eines Keramikmaterials, aufweisend 20 bis 100 Gew.-% Titandioxid, auf die Oberfläche bis zu wenigstens 100 µm Dicke aufweist, so dass die aufgespritzte Beschichtung ein dunkelgraues oder schwarzes Aussehen hat.

11. Verfahren wie in Anspruch 10 beansprucht, wobei das Keramikmaterial Titandioxid und wenigstens ein anderes Keramikmaterial aufweist, vorzugsweise wenigstens eines von Zirkoniumdioxid, Chromdioxid, Aluminiumdioxid und Magnesiumzirkonat.

12. Verfahren nach Anspruch 10 oder 11, wobei das Plasmaspritzen Stickstoff-Plasmaspritzen ist.

13. Verfahren nach Anspruch 10, Anspruch 11 oder Anspruch 12, wobei das Verfahren ferner das Aufbringen einer Haftschicht auf die Oberfläche vor dem Aufbringen der Wärmesperre aufweist, wobei die Haftschicht vorzugsweise ein Metall oder eine Metalllegierung ist und bevorzugter Nickel ist oder Nickel enthält.

14. Verwendung von plastmagespritztem Titandioxid in Alleinstellung oder in Kombination mit einem anderen Keramikmaterial mit einem Titandioxidgehalt von wenigstens 20 Gew.-% in einer Beschichtung von wenigstens 100 µm Dicke als Wärmesperre auf einem Artikel aus Metall, wobei es ein Fahrzeugauspuff oder ein Motorradauspuff ist, wobei die Beschichtung plasmagespritzt ist, um ein dunkelgraues oder schwarzes Aussehen zu erreichen.

## Revendications

1. Article doté d'une barrière thermique comprenant un revêtement de matériau céramique comprenant 20 à 100 % en poids de dioxyde de titane, dans lequel la barrière thermique est un revêtement pulvérisé au plasma présentant un aspect gris foncé ou noir, l'épaisseur du revêtement étant d'au moins 100 micromètres, l'article étant en métal et étant un tuyau d'échappement de voiture ou un échappement de moto.

2. Article selon la revendication 1, dans lequel le revêtement comprend un revêtement de dioxyde de titane uniquement.

3. Article selon la revendication 1, dans lequel le revêtement présente environ plus de 30 % en poids de dioxyde de titane, et de préférence présente au moins 50 % en poids de dioxyde de titane.

4. Article selon la revendication 1, 2 ou 3, dans lequel le revêtement comprend du dioxyde de titane et au moins un autre matériau céramique, et l'autre matériau céramique comprend de préférence au moins un élément parmi le dioxyde de zirconium, le dioxyde de chrome, le dioxyde d'aluminium et le zirconate de magnésium.

5. Article selon l'une quelconques des revendications précédentes, dans lequel la barrière thermique est un revêtement pulvérisé au plasma.

6. Article selon l'une quelconque des revendications précédentes, dans lequel la barrière thermique présente différentes épaisseurs à différents endroits pour fournir différents degrés de protection contre la chaleur.

7. Article selon l'une quelconque des revendications précédentes, dans lequel la barrière thermique ne présente pas une épaisseur supérieure à 500 micromètres.

8. Article selon l'une quelconque des revendications précédentes, dans lequel l'article est en acier.

9. Article selon l'une quelconque des revendications précédentes, dans lequel l'article comprend au moins une couche intermédiaire sous la barrière thermique, de préférence ladite ou une couche intermédiaire étant un métal ou un alliage métallique, et plus préférablement la couche intermédiaire étant ou contenant du nickel.

10. Procédé d'application d'une barrière thermique sur une surface d'un article métallique, l'article étant un tuyau d'échappement de voiture ou un échappement de moto, le procédé comprenant la pulvérisation au plasma sur la surface d'un matériau céramique comprenant 20 à 100 % en poids de dioxyde de titane sur une épaisseur d'au moins 100 micromètres de sorte que le revêtement pulvérisé présente un aspect gris foncé ou noir.

11. Procédé selon la revendication 10, dans lequel le matériau céramique comprend du dioxyde de titane et au moins un autre matériau céramique, de préférence au moins un élément parmi le dioxyde de zirconium, le dioxyde de chrome, l'oxyde d'aluminium et le zirconate de magnésium.

12. Procédé selon la revendication 10 ou la revendication 11, dans lequel la pulvérisation de plasma est une pulvérisation de plasma d'azote.

13. Procédé selon la revendication 10, la revendication 11 ou la revendication 12, dans lequel le procédé comprend en outre l'application d'un revêtement de liaison sur la surface avant d'appliquer la barrière thermique, le revêtement de liaison étant de préférence un métal ou un alliage métallique, et plus préférablement étant ou contenant du nickel.

14. Utilisation de dioxyde de titane pulvérisé au plasma, seul ou en combinaison avec un autre matériau céramique, à une teneur en dioxyde de titane d'au moins 20 % en poids, dans un revêtement d'au moins 100 micromètres d'épaisseur, comme une barrière thermique sur un article en métal qui est un tuyau d'échappement de voiture ou un échappement de moto, le revêtement étant pulvérisé au plasma de manière à obtenir un aspect gris foncé ou noir.
